# EUROPEAN PATENT SPECIFICATION

(11) **EP 2 760 595 B1**
(45) Date of publication and mention of the grant of the patent: **25.07.2018**
(21) Application number: 12835615.1
(22) Date of filing: 16.08.2012
(51) Int. Cl.: B05D 3/04, C23C 18/24, C23C 18/30, C23C 18/20, C23C 18/32

(54) **TREATMENT OF PLASTIC SURFACES AFTER ETCHING IN NITRIC ACID CONTAINING MEDIA**
BEHANDLUNG VON KUSTSTOFFOBERFLÄCHEN NACH DEM ÄTZEN IN SALPETERSÄUREHALTIGEN MEDIEN
TRAITEMENT DES SURFACES EN PLASTIQUE APRÈS LA GRAVURE DANS UNE SUBSTANCE CONTENANT DE L'ACIDE NITRIQUE

(30) Priority: 29.09.2011 US 201113248550
(43) Date of publication of application: 06.08.2014
(73) Proprietor: MacDermid Acumen, Inc., Waterbury, CT 06702 (US)
(72) Inventor: CHAPANERI, Roshan, V., Foleshill, Coventry CV6 5JH (GB); WALL, Anthony, Oldbury, West Midlands B68 9QS (GB); PEARSON, Trevor, Cradley Heath West Midlands B64 7HR (GB); HERDMAN, Roderick, D., Tamworth Staffordshire B78 2JQ (GB)
(74) Representative: Jenkins, Peter David
(86) International application number: PCT/US2012/051136
(87) International publication number: WO 2013/048635

(56) References cited:
- EP-A1- 0 913 498
- EP-A1- 2 149 622
- EP-A2- 0 187 962
- EP-A2- 0 321 856
- DE-A1- 19 918 833
- US-A- 3 899 617
- US-A- 3 899 617
- US-A- 5 160 600
- US-A- 5 160 600
- US-A1- 2009 205 969
- US-A1- 2010 120 962

## Description

### FIELD OF THE INVENTION

The present invention relates generally to the treatment of plastic surfaces following etching in an acidic solution containing nitrate ions.

### BACKGROUND OF THE INVENTION

For many years, processes have been available to facilitate the deposition of electrodeposited metals onto plastic substrates. A typical process involves the steps of:
(1) etching the plastic in a suitable etching solution such that the surface of the plastic becomes roughened and wetted so that the subsequently applied deposit has good adhesion;
(2) activating the surface of the plastic using a colloidal or ionic solution of a metal capable of initiating the deposition of an autocatalytically applied metal coating of typically copper or nickel;
(3) depositing a thin layer of autocatalytically applied metal; and
(4) carrying out electrodeposition of metal onto the metallized plastic substrate.
Typically, layers of copper, nickel and/or chromium are applied to produce the final article.

The most widely used plastic substrates include acrylonitrile/butadiene/styrene copolymers (ABS) or ABS blended with polycarbonate (ABS/PC). These materials are readily formed into components by the process of injection molding. ABS comprises a relatively hard matrix of acrylonitrile/styrene copolymer and the butadiene polymerizes to form a separate phase. It is this softer phase of polybutadiene (which contains double bonds in the polymer backbone) which can be readily etched using various techniques.

Traditionally, the etching has been carried out using a mixture of chromic and sulfuric acids which must be operated at an elevated temperature. The chromic acid is capable of dissolving the polybutadiene phase of the ABS by oxidation of the double bonds in the backbone of the polybutadiene polymer, and this has proven to be reliable and effective over a wide range of ABS and ABS/PC plastics. However, the use of chromic acid is becoming increasingly regulated because of its toxicity and carcinogenic nature. For this reason, there has been a considerable amount of research into other means of etching ABS and ABS/PC plastics.

There are a number of approaches possible in order to attempt to achieve this. For example, acidic permanganate is capable of oxidizing the double bonds in the polybutadiene. Chain scission can then be achieved by further oxidation with periodate ions. Ozone is also capable of oxidizing polybutadiene and this approach has also been attempted. However, ozone is extremely dangerous to use and is also highly toxic. Likewise, sulfur trioxide can be successfully utilized to etch ABS, but this cannot be successfully achieved on a typical plating line. Other examples of prior art techniques for etching ABS plastics without the use of chromic acid can be found in U.S. Pat. Pub. No. 2005/0199587 to Bengston, U.S. Pat. Pub. No. 2009/0092757 to Sakou and U.S. Pat. No. 5,160,600 to Gordhanbai. However, none of these methods have achieved widespread commercial acceptance.

EP2149622 describes a pretreatment process for electroless plating of a resin molded article, comprising etching the resin molded article using a manganate salt-containing etching solution, and then bringing the resin molded article into contact with an aqueous solution containing a reducing compound and an inorganic acid.

US5160600 describes a process of electroless plating of polymers containing units derived from at least one member of the group consisting of acrylonitrile, butadiene and styrene, is carried out in an environment free of chromium ions, by the sequential steps of roughening and activating the surface of the polymer by contacting the same with an aqueous solution of a concentrated sulfur acid, of concentrated nitric acid or of concentrated phosphoric acid, in the presence of noble metal ion and an oxidant selected from the group consisting of nitric acid, hydrogen peroxide and persulfates.

DE19918833 describes electroplating of a non-conductive substrate involves contact with an electroless reduction copper bath after precious metal activation and nucleation and before electroplating.

EP0187962 describes a catalytic adsorbate suspended in an aqueous solution comprising reduced catalytic metal on an organic suspending agent where the reduced catalytic metal has a maximum dimension not exceeding 500 angstroms and the organic suspending agent is one capable of complexing with ions of the catalytic metal.

US3899617 describes ABS resin surfaces that are etched by contact with a strong acid oxidizing solution, and then post-etched by contact with an alkanol amine aqueous solution.

EP0321856 describes the use of certain quaternary salts of di- and/or trialkanolamines, which salts are soluble in an aqueous application bath, as conditioners for the pretreatment of nonmetallic surfaces of mouldings before the nucleation thereof for a subsequent chemical metallisation.

Thus, there remains a need in the art for an improved process of etching plastics without chromic acid, while continuing to utilize a conventional activation process containing a palladium colloid followed by electroless nickel.

### SUMMARY OF THE INVENTION

It is an object of the present invention to provide a process for etching plastics without the use of chromic acid.

It is another object of the present invention to provide a process for etching acrylonitrile/butadiene/styrene copolymers without the use of chromic acid.

It is still another object of the present invention to provide an improved conditioning treatment for conditioning the surfaces of an etched plastic.

To that end, the present invention relates to a method of treating a plastic substrate to accept electroless plating thereon according to claim 1, the method comprising the steps of:
a) etching a surface of the plastic substrate by contacting the plastic substrate with an acidic solution containing nitrate ions and oxidizing metal ions, wherein the oxidizing metal ions are produced by electrochemical oxidation, wherein the acidic solution comprises silver nitrate and nitric acid;
b) contacting the etched plastic substrate with a conditioning solution comprising an aqueous solution comprising ammonia, an amine or combinations thereof;
c) activating the plastic substrate comprising contacting the plastic substrate with an activation solution comprising palladium; and
d) contacting the activated plastic substrate with an electroless metal plating solution to deposit metal thereon, wherein the electroless metal plating solution comprises electroless nickel.
Further features of the invention are defined in the dependent claims.

### BRIEF DESCRIPTION OF THE FIGURES

Figure 1 depicts an infra-red analysis obtained from untreated ABS.
Figures 2A and 2B depict an infra-red analysis obtained from ABS treated with a chromic acid/sulfuric acid etch solution of the prior art.
Figures 3A and 3B depict an infra-red analysis obtained from ABS treated with an acidic solution of nitrate and silver ions.
Figures 4A and 4B depict an infra-red analysis obtained from ABS treated with an acidic solution of nitrate and silver ions and then post-treated in an ammonia solution.

### DETAILED DESCRIPTION OF THE PREFERRED EMBODIMENTS

In preliminary experiments using nitric acid/silver(II) etch compositions, the inventors of the present invention discovered that although this etch composition can be used to effectively etch an ABS or ABS/PC plastic to give an excellent surface topography, the subsequent catalysis of the surface could not be achieved and there was no deposition of nickel when the components were subsequently immersed in the electroless nickel plating process. Examination of the surface of the plastic using infrared spectroscopy indicates that the surface of the plastic has been chemically altered to some degree. New peaks were found following the etching stage, which almost disappeared when the plastic was immersed in hot water (80°C) for 10 minutes. However, even though the surface of the plastic had apparently reverted in composition to something similar to its original composition, palladium adsorption and subsequent catalyzation of the surface could not be achieved.

Surprisingly, the inventors of the present invention have discovered that immersing the etched plastic in a solution containing amines can condition the surface so that palladium adsorption can be achieved. Without wishing to be bound by theory, the inventors consider that it is possible that the amines are adsorbed onto the surface of the etched plastic, thus imparting a positive charge on the surface of the plastic when immersed into the acidic palladium colloid solution. With primary, secondary and tertiary amines, this positive charge is most likely formed by protonation of the amines, and with quaternary amines, the positive charge is already present on the amine.

The inventors have also found, through infrared spectroscopy, that an etched plastic can be modified with an amine-based post treatment. In addition to the disappearance of the peaks introduced following the etching stage, a new functional group appears to have been introduced. The composition of the invention conditions the surface of the plastic so that effective palladium adsorption can be achieved in order to catalyze the subsequent deposition of autocatalytic metal deposits.

According to the present invention, a method is provided for the catalysis and subsequent metallization of plastics which have been etched in nitric acid containing solutions. The method of the invention comprises the following steps:
a) etching a surface of the plastic substrate by contacting the plastic substrate with an acidic solution containing nitrate ions and oxidizing metal ions, wherein the oxidizing metal ions are produced by electrochemical oxidation, wherein the acidic solution comprises silver nitrate and nitric acid;
b) contacting the etched plastic substrate with a conditioning solution comprising an aqueous solution comprising ammonia, an amine or combinations thereof;
c) activating the plastic substrate comprising contacting the plastic substrate with an activation solution comprising palladium; and
d) contacting the activated plastic substrate with an electroless metal plating solution to deposit metal thereon, wherein the electroless metal plating solution comprises electroless nickel
Following the above steps, the metallized component can be electroplated in the usual manner.

The acidic etching solution comprises silver nitrate and nitric acid. In addition, other mineral acids such as sulfuric acid may also be added to the composition. The acidic etching solution may also contain oxidizing metallic ions of metals including, for example, manganese, cobalt, cerium and combinations thereof, preferably in their highest oxidation state. These ions are produced by a process of electrochemical oxidation. In addition, if desired, a wetting agent may also be added to the acidic etching solution. One suitable wetting agent is available from MacDermid, Inc. under the trade name Macuplex STR.

Thereafter, the etched plastic substrate is contacted with the conditioning solution. In one preferred embodiment the etched plastic substrate is immersed in the conditioning solution. The concentration of amines or ammonia in the aqueous conditioning solution is not critical but is preferably within the range of about 5 to about 100 g/L, more preferably in the range of about 10 to about 50 g/L. The pH of the solution may be from 0 to 14, but is preferably in the range of 6-12.

As discussed above, the amine may be a primary, secondary, tertiary or quarternary amine. In the alternative, the solution may comprise ammonia instead of the amine. In addition, it is also possible to use a combination of different amines or a combination of an amine with ammonia in the conditioning solution of the invention.

Suitable primary amines include, for example, monoethylamine, mono-n-propylamine, iso-propylamine, mono-n-butylamine, iso-butylamine, monoethanolamine, neopentanolamine, 2-aminopropanol, 3-aminopropanol, 2-hydroxy-2'(aminopropoxy) ethylether, 1-aminopropanol, monoisopropanolamine, diethylaminopropylamine, aminoethyl ethanolamine and combinations of the foregoing. In a preferred embodiment, the primary amine comprises monoisopropanolamine or diethylenetriamine.

Suitable secondary amines include, for example, diethylamine, dibutylamine, diethanolamine, methylethylamine, di-n-propanolamine, di-iso-propanolamine, N-methylethanolamine, N-ethylethanolamine, N-methylethanolamine, di-isopropanolamine, diethylenetriamine, triethylenetetramine, tetraethylenepentamine and combinations of the foregoing. In a preferred embodiment, the secondary amine comprises di-ethanolamine or diethylenetriamine.

Suitable tertiary amines include, for example, N,N-dimethylethanolamine, triethylamine, trimethylamine, triisopropylamine, methyldiethanolamine, triethanolamine, and combinations of one or more of the foregoing. In a preferred embodiment, the tertiary amine comprises N,N-dimethylethanolamine.

Quarternary amines are also generally suitable, including quarternary (poly) amines. Suitable quarternary amines also include polymeric quarternary amines having the general formula:

Wherein:
R¹, R², R³ and R⁴ independently can be the same or different and may be selected from-CH₃, -CH₂CH₃, -CH(CH₃)₂ or -CH₂CH₂OH;
R⁵ is -CH₂CH₂-, -CH₂CH₂CH₂-, -CH₂CH₂CH₂CH₂-, -CH₂CHOHCH₂- or -CH₂CH₂OCH₂CH₂;
X and Y can be the same or different and are selected from Cl, Br, and I;
v and u can be the same or different and each can be 1 to 7; and
n is 2 to about 200.

In one embodiment the polymeric quaternary amine is Mirapol™ WT (available from Rhodia) in which in the above formula:
R¹, R², R³ and R⁴ are each CH₃;
R⁵ is -CH₂CH₂OCH₂CH₂;
v and u are 3;
X and Y are Cl; and
n is an average of about 6.

Other suitable polymeric amines include polyethyleneimines such as Lugalvan™ G35 available from BASF.

The invention can now be illustrated by reference to the following non-limiting examples:
The following details apply to the examples:
POLYLAC™ PA727 is a commercial grade of acrylonitrile butadiene styrene (ABS) manufactured by Chi Mei, Inc., Taiwan.

The following products described in the examples are available from MacDermid, Inc. and were used in accordance with their product data sheets.

| **Product** | **Description** |
|---|---|
| ND7 Supreme™ | Pre-etch cleaning/decreasing solution |
| Macuplex™ STR | Wetting agent |
| Macuplex™ 9338 | Neutralizing treatment for hexavalent chromium |
| Macuplex™ D-34C | Activating solution based on colloidal suspension of metallic palladium particles in a stannous chloride medium |
| Macuplex™ 9369 | Post-activator acidic treatment to improve the autocatalytic nature of the activated surface |
| Macuplex™ J-64 | Electroless nickel plating bath |

Infra-red (IR) instrument and analysis details:
Instrument - PerkinElmer spectrum 100 FTIR spectrometer
Analysis details:
- Attenuated total reflectance (ATR) mode
- Wavenumber range - 4000-6000 cm⁻¹
- Number of scans - 8

### Comparative example 1:

Untreated POLYLAC™ PA727 The Infra-Red analysis obtained from untreated ABS is shown in Figure 1.

### Comparative example 2:

POLYLAC™ PA727 processed through a chromic acid/sulfuric etch solution of the prior art.

| **Process** | **Details** | **Temperature (°C)** | **Time** |
|---|---|---|---|
| ND7 Supreme™ | | 50 | 2 minutes |
| Water rinse | | Ambient | 1 minute |
| Etch | 4 M chromic acid | 68 | 7 minutes |
| | 3.6 M sulfuric acid | | |
| | 1 ml/l Macuplex STR | | |
| Water rinse | | Ambient | 2 minutes |
| Macuplex™ 9338 | | 30 | 2 minutes |
| Water rinse | | Ambient | 1 minute |
| Dry | | | |
| Infra-Red analysis | | | |

The infra-red spectrum obtained is shown in Figures 2A and 2B.

In the following examples 3-9, the chromium free etch solution is contained in a 2-compartment glass cell separated by a glass frit, with the etching solution being the anolyte (the catholyte being of the same composition with the exception of the silver nitrate being absent in the catholyte). The anode and cathode materials were platinized titanium mesh and the anodic current density used was 32.5 mA/cm². This system was used to electrochemically oxidize the silver ions to the +2 oxidation state.

A mechanical stirrer bar was used to provide agitation and the cell was electrolyzed by a minimum of two hours before use in order to generate a significant quantity of silver (II) ions.

### Example 3.

Example 3 illustrates an ABS substrate processed through non-chrome etch solution:

| **Process** | **Details** | **Temperature (°C)** | **Time** |
|---|---|---|---|
| ND7 Supreme™ | | 50 | 2 minutes |
| Water rinse | | Ambient | 1 minute |
| Etch | 0.1 M AgNO₃ | 50 | 6 minutes |
| | 9 M HNO₃ | | |
| | 7 ml/l Macuplex STR | | |
| Water rinse | | Ambient | 2 minutes |
| Dry | | | |
| Infra-Red analysis | | | |

The infra-red spectrum obtained is shown in Figure 3A and 3B. Figures 3A and 3B depict the FTIR spectrum of POLYLAC™ PA727 etched in an acidic solution containing nitrate ions and silver ions. Figure 3A shows the results at 4000-600 cm⁻¹ and Figure 3B shows the results at 2000-600 cm⁻¹. The "*" in the Figures 3A and 3B indicate peaks that have appeared due to the etching process.

### Example 4:

Example 4 illustrates an ABS substrate processed through a non-chrome etch solution and an ammonia post-treatment solution.

| **Process** | **Details** | **Temperature (°C)** | **Time** |
|---|---|---|---|
| ND7 Supreme™ | | 50 | 2 minutes |
| Water rinse | | Ambient | 1 minute |
| Etch | Same as Example 3 | 50 | 6 minutes |
| Water rinse | | Ambient | 2 minutes |
| Ammonia treatment | 40 ml/l of 0.880SG ammonia solution (or 0.68M NH₃) | 50 | 5 minutes |
| Water rinse | | Ambient | 1 minute |
| Dry | | | |
| Infra-Red analysis | | | |

The infra-red spectrum obtained is shown in Figures 4A and 4B. Figures 4A and 4B depict the FTIR spectrum of POLYLAC™ PA727 etched in an acidic solution containing nitrate ions and silver ions and post treated in an ammonia solution. Figure 4A shows the results at 4000-600 cm⁻¹ and Figure 4B shows the results at 2000-600 cm⁻¹. As can be seen in Figures 4A and 4B, there is an absence of the peaks introduced in Example 3. In this example, the "*" in Figure 4B indicates a new peak introduced by treatment with an amine.

### Example 5:

Example 5 illustrates an ABS substrate processed through a non-chrome etch solution an ammonia post-treatment solution and up to the electroless nickel stage:

| **Process** | **Details** | **Temperature (°C)** | **Time** |
|---|---|---|---|
| ND7 Supreme™ | | 50 | 2 minutes |
| Water rinse | | Ambient | 1 minute |
| Etch | Same as Example 3 | 50 | 6 minutes |
| Water rinse | | Ambient | 2 minutes |
| Ammonia treatment | 40 ml/l of 0.880 SG ammonia solution | 50 | 5 minutes |
| Water rinse | | Ambient | 1 minute |
| Acid rinse | 2.8M HCl | Ambient | 1 minute |
| Macuplex™ D-34C | | 27 | 3 minutes |
| Water rinse | | Ambient | 1 minute |
| Macuplex™ 9369 | | 48 | 2 minutes |
| Water rinse | | Ambient | 1 minute |
| Macuplex™ J-64 | | 32 | 7 minutes |
| Water rinse | | Ambient | 1 minute |
| Dry | | | |

The result was full electroless nickel metallization.

### Example 6:

Example 6 illustrates an ABS substrate processed through a non-chrome etch solution, deionized water post-treatment solution and up to the electroless nickel stage:

| **Process** | **Details** | **Temperature (°C)** | **Time** |
|---|---|---|---|
| ND7 Supreme™ | | 50 | 2 minutes |
| Water rinse | | Ambient | 1 minute |
| Etch | 0.1 M AgNO₃ | 55 | 6 minutes |
| | 6 M HNO₃ | | |
| | 6 M H₂SO₄ | | |
| | 1 ml/l Macuplex STR | | |
| Water rinse | | Ambient | 5 minutes |
| Hot water rinse | | 80 | 10 minutes |
| Water rinse | | Ambient | 1 minute |
| Acid rinse | 2.8 M HCl | Ambient | 1 minute |
| Macuplex™ D-34C | | 27 | 3 minutes |
| Water rinse | | Ambient | 1 minute |
| Macuplex™ 9369 | | 48 | 2 minutes |
| Water rinse | | Ambient | 1 minute |
| Macuplex™ J-64 | | 32 | 7 minutes |
| Water rinse | | Ambient | 1 minute |
| Dry | | | |

The result was no electroless nickel metallization.

### Example 7:

Example 7 illustrates an ABS substrate processed through a non-chrome etch solution, a N,N-dimethylethanolamine post treatment solution and up to the electroless nickel stage:

| **Process** | **Details** | **Temperature (°C)** | **Time** |
|---|---|---|---|
| ND7 Supreme™ | | 50 | 2 minutes |
| Water rinse | | Ambient | 1 minute |
| Etch | Same as Example 6 | 55 | 6 minutes |
| Water rinse | | Ambient | 2 minutes |
| Amine treatment | 10 g/L N,N-dimethylethanolamine | 80 | 10 minutes |
| Water rinse | | Ambient | 1 minute |
| Acid rinse | 2.8 M HCl | Ambient | 1 minute |
| Macuplex™ D-34C | | 27 | 3 minutes |
| Water rinse | | Ambient | 1 minute |
| Macuplex™ 9369 | | 48 | 2 minutes |
| Water rinse | | Ambient | 1 minute |
| Macuplex™ J-64 | | 32 | 7 minutes |
| Water rinse | | Ambient | 1 minute |
| Dry | | | |

The result was full electroless nickel metallization.

### Example 8:

Example 8 illustrates an ABS substrate processed through a non-chrome etch solution, a diethylene triamine post treatment solution and up to the electroless nickel stage:

| **Process** | **Details** | **Temperature (°C)** | **Time** |
|---|---|---|---|
| ND7 Supreme™ | | 50 | 2 minutes |
| Water rinse | | Ambient | 1 minute |
| Etch | 0.1 M AgNO₃ | 55 | 12 minutes |
| | 6 M HNO₃ | | |
| | 3 M H₂SO₄ | | |
| Water rinse | | Ambient | 2 minutes |
| Amine treatment | 15 g/L diethylene triamine | 50 | 5 minutes |
| Water rinse | | Ambient | 1 minute |
| Acid rinse | 2.8 M HCl | Ambient | 1 minute |
| Macuplex™ D-34C | | 27 | 3 minutes |
| Water rinse | | Ambient | 1 minute |
| Macuplex™ 9369 | | 48 | 2 minutes |
| Water rinse | | Ambient | 1 minute |
| Macuplex™ J-64 | | 32 | 7 minutes |
| Water rinse | | Ambient | 1 minute |
| Dry | | | |

The result was full electroless nickel metallization.

### Example 9:

Example 9 illustrates an ABS substrate processed through a non-chrome etch solution, a polymeric quaternary amine post treatment solution and up to the electroless nickel stage:

| **Process** | **Details** | **Temperature (°C)** | **Time** |
|---|---|---|---|
| ND7 Supreme™ | | 50 | 2 minutes |
| Water rinse | | Ambient | 1 minute |
| Etch | Same as Example 8 | 50 | 6 minutes |
| Water rinse | | Ambient | 2 minutes |
| Amine treatment | 15 g/L Mirapol WT, a polymeric quaternary amine available from Rhodia | 50 | 5 minutes |
| Water rinse | | Ambient | 1 minute |
| Acid rinse | 2.8 M HCl | Ambient | 1 minute |
| Macuplex™ D-34C | | 27 | 3 minutes |
| Water rinse | | Ambient | 1 minute |
| Macuplex™ 9369 | | 48 | 2 minutes |
| Water rinse | | Ambient | 1 minute |
| Macuplex™ J-64 | | 32 | 7 minutes |
| Water rinse | | Ambient | 1 minute |
| Dry | | | |

The result was full electroless nickel metallization.

## Claims

1. A method of treating a plastic substrate to accept electroless plating thereon, the method comprising the steps of:
a) etching a surface of the plastic substrate by contacting the plastic substrate with an acidic solution containing nitrate ions and oxidizing metal ions, wherein the oxidizing metal ions are produced by electrochemical oxidation, wherein the acidic solution comprises silver nitrate and nitric acid;
b) contacting the etched plastic substrate with a conditioning solution comprising an aqueous solution comprising ammonia, an amine or combinations thereof;
c) activating the plastic substrate comprising contacting the plastic substrate with an activation solution comprising palladium; and
d) contacting the activated plastic substrate with an electroless metal plating solution to deposit metal thereon, wherein the electroless metal plating solution comprises electroless nickel.

2. The method according to claim 1, wherein the acidic solution comprises a wetting agent.

3. The method according to claim 1, comprising the step of immersing the plastic substrate into an acid rinse after step (b).

4. The method according to claim 1, wherein the amine comprises at least one of a primary amine, a secondary amine, a tertiary amine and a quaternary amine.

5. The method according to claim 4, wherein the primary amine is selected from the group consisting of monoethylamine, mono-n-propylamine, iso-propylamine, mono-n-butylamine, iso-butylamine, monoethanolamine, neopentanolamine, 2-aminopropanol, 3-aminopropanol, 2-hydroxy-2' (aminopropoxy)ethylether, 1-aminopropanol,monoisopropanolamine, diethylaminopropylamine, 2-aminoethylethanolamine and combinations of the foregoing, optionally wherein the primary amine comprises monoisopropanol amine.

6. The method according to claim 4, wherein the secondary amine is selected from the group consisting of diethylamine, dibutylamine, diethanolamine, methylethylamine, di-n-propanolamine, iso-propanolamine, N-methylethanolamine, diethylenetriamine, N-ethylethanolamine, N-methylethanolamine, di-isopropanol amine, and combinations of the foregoing, optionally wherein the secondary amine comprises diethanolamine, further optionally wherein the secondary amine comprises diethylenetriamine.

7. The method according to claim 4, wherein the tertiary amine is selected from the group consisting of N,N-dimethylethanolamine, triethylamine, trimethylamine, triisopropylamine, methyldiethanolamine, triethanolamine and combinations of one or more of the foregoing, optionally wherein the tertiary amine comprises N,N-dimethylethanolamine.

8. The method according to claim 4, wherein the quaternary amine comprises a polymeric quaternary amine having the general formula: wherein:
R¹, R², R³ and R⁴ independently can be the same or different and may be selected from-CH₃, -CH₂CH₃, -CH(CH₃)₂ or -CH₂CH₂OH;
R⁵ is -CH₂CH₂-, -CH₂CH₂CH₂-, -CH₂CH₂CH₂CH₂-, -CH₂CHOHCH₂- or -CH₂CH₂OCH₂CH₂;
X and Y can be the same or different and are selected from Cl, Br, and I;
v and u can be the same or different and each can be 1 to 7; and
n is 2 to 200, optionally wherein in the polymeric quaternary amine, R¹, R², R³ and R⁴ are each CH₃;
R⁵ is -CH₂CH₂OCH₂CH₂;
v and u are 3;
X and Y are Cl; and
n is an average of 6.

9. The method according to claim 1 wherein the concentration of the amine and/or the ammonia in the conditioning solution is between 5 and 100 g/L, optionally wherein the concentration of the amine and/or the ammonia in the conditioning solution is between 10 and 50 g/L.

10. The method according to claim 1, wherein the conditioning solution has a pH of between 0 to 14, optionally wherein the conditioning solution has a pH of between 6 and 12.

11. The method according to claim 1, further comprising the step of contacting the activated plastic substrate with an acid treatment prior to step (d).

## Patentansprüche

1. Verfahren zur Behandlung eines Kunststoffsubstrats, um chemische Abscheidung darauf zuzulassen, wobei das Verfahren die folgenden Schritte umfasst:
a) Ätzen einer Oberfläche des Kunststoffsubstrats durch Inkontaktbringen des Kunststoffsubstrats mit einer sauren Lösung, die Nitrationen und oxidierende Metallionen enthält, wobei die oxidierenden Metallionen durch elektrochemische Oxidation produziert werden, wobei die saure Lösung Silbernitrat und Salpetersäure umfasst;
b) Inkontaktbringen des geätzten Kunststoffsubstrats mit einer Konditionierungslösung, die eine wässrige Lösung umfasst, die Ammoniak, ein Amin oder Kombinationen davon umfasst;
c) Aktivieren des Kunststoffsubstrats, das das Inkontaktbringen des Kunststoffsubstrats mit einer Aktivierungslösung umfasst, die Palladium umfasst; und
d) Inkontaktbringen des aktivierten Kunststoffsubstrats mit einer chemischen Metallabscheidungslösung, um Metall darauf abzuscheiden, wobei die chemische Metallabscheidungslösung chemischen Nickel umfasst.

2. Verfahren nach Anspruch 1, wobei die saure Lösung ein Benetzungsmittel umfasst.

3. Verfahren nach Anspruch 1, das den Schritt des Eintauchens des Kunststoffsubstrats in ein saures Spülbad nach Schritt (b) umfasst.

4. Verfahren nach Anspruch 1, wobei das Amin mindestens eines von einem primären Amin, einem sekundären Amin, einem tertiären Amin und einem quaternären Amin umfasst.

5. Verfahren nach Anspruch 4, wobei das primäre Amin aus der Gruppe bestehend aus Monoethylamin, Mono-n-propylamin, Isopropylamin, Mono-n-butylamin, Isobutylamin, Monoethanolamin, Neopentanolamin, 2-Aminopropanol, 3-Aminopropanol, 2-Hydroxy-2'-(aminopropoxy)ethylether, 1-Aminopropanol, Monoisopropanolamin, Diethylaminopropylamin, 2-Aminoethylethanolamin und Kombinationen der vorstehenden ausgewählt ist, gegebenenfalls wobei das primäre Amin Monoisopropanolamin umfasst.

6. Verfahren nach Anspruch 4, wobei das sekundäre Amin aus der Gruppe bestehend aus Diethylamin, Dibutylamin, Diethanolamin, Methylethylamin, Di-n-propanolamin, Isopropanolamin, N-Methylethanolamin, Diethylentriamin, N-Ethylethanolamin, N-Methylethanolamin, Diisopropanolamin und Kombinationen der vorstehenden ausgewählt ist, gegebenenfalls wobei das sekundäre Amin Diethanolamin umfasst, weiterhin gegebenenfalls wobei das sekundäre Amin Diethylentriamin umfasst.

7. Verfahren nach Anspruch 4, wobei das tertiäre Amin aus der Gruppe bestehend aus N,N-Dimethylethanolamin, Triethylamin, Trimethylamin, Triisopropylamin, Methyldiethanolamin, Triethanolamin und Kombinationen von einem oder mehreren der vorstehenden ausgewählt ist, gegebenenfalls wobei das tertiäre Amin N,N-Dimethylethanolamin umfasst.

8. Verfahren nach Anspruch 4, wobei das quaternäre Amin ein polymeres quaternäres Amin mit der folgenden allgemeinen Formel umfasst: wobei:
R¹, R², R³ und R⁴ unabhängig gleich oder verschieden sein können und aus -CH₃, -CH₂CH₃, -CH(CH₃)₂ oder -CH₂CH₂OH ausgewählt sein können;
R⁵ -CH₂CH₂-, -CH₂CH₂CH₂-, -CH₂CH₂CH₂CH₂-, -CH₂CHOHCH₂- oder -CH₂CH₂OCH₂CH₂ ist;
X und Y gleich oder verschieden sein können und aus Cl, Br und I ausgewählt sind;
v und u gleich oder verschieden sein können und jeweils 1 bis 7 sein können und
n 2 bis 200 ist, gegebenenfalls wobei in dem polymeren quaternären Amin
R¹, R², R³ und R⁴ jeweils CH₃ sind;
R⁵ -CH₂CH₂OCH₂CH₂ ist;
v und u 3 sind;
X und Y Cl sind und
n durchschnittlich 6 ist.

9. Verfahren nach Anspruch 1, wobei die Konzentration des Amins und/oder des Ammoniaks in der Konditionierungslösung zwischen 5 und 100 g/L liegt, gegebenenfalls wobei die Konzentration des Amins und/oder des Ammoniaks in der Konditionierungslösung zwischen 10 und 50 g/L liegt.

10. Verfahren nach Anspruch 1, wobei die Konditionierungslösung einen pH-Wert zwischen 0 und 14 aufweist, gegebenenfalls wobei die Konditionierungslösung einen pH-Wert zwischen 6 und 12 aufweist.

11. Verfahren nach Anspruch 1, das weiterhin den Schritt des Inkontaktbringens des aktivierten Kunststoffsubstrats mit einer Säurebehandlung vor Schritt (d) umfasst.

## Revendications

1. Procédé de traitement d'un substrat en plastique pour qu'il soit possible d'effectuer un dépôt autocatalytique sur celui-ci, le procédé comprenant les étapes suivantes :
(a) gravure d'une surface du substrat en plastique par mise en contact du substrat en plastique avec une solution acide contenant des ions nitrates et des ions métalliques oxydants, où les ions métalliques oxydants sont produits par oxydation électrochimique et où la solution acide comprend du nitrate d'argent et de l'acide nitrique ;
(b) mise en contact du substrat en plastique gravé avec une solution de conditionnement comprenant une solution aqueuse qui comprend de l'ammoniaque, une amine ou des combinaisons de celles-ci ;
(c) activation du substrat en plastique qui comprend la mise en contact du substrat en plastique avec une solution d'activation comprenant du palladium ; et
(d) mise en contact du substrat en plastique activé avec une solution de dépôt autocatalytique d'un métal pour déposer un métal sur celui-ci, où la solution de dépôt autocatalytique d'un métal comprend du nickel autocatalytique.

2. Procédé selon la revendication 1, où la solution acide comprend un agent mouillant.

3. Procédé selon la revendication 1 comprenant l'étape d'immersion du substrat en plastique dans un bain de rinçage acide après l'étape (b).

4. Procédé selon la revendication 1, où l'amine comprend au moins une parmi une amine primaire, une amine secondaire, une amine tertiaire et une amine quaternaire.

5. Procédé selon la revendication 4, où l'amine primaire est sélectionnée dans le groupe consistant en les suivantes : monoéthylamine, mono-n-propylamine, iso-propylamine, mono-n-butylamine, iso-butylamine, monoéthanolamine, néopentanolamine, 2-aminopropanol, 3-aminopropanol, éther 2-hydroxy-2'(aminopropoxy)éthylique, 1-aminopropanol, monoisopropanolamine, diéthylaminopropylamine, 2-aminoéthyléthanolamine et combinaisons de celles-ci, éventuellement où l'amine primaire comprend la monoisopropanolamine.

6. Procédé selon la revendication 4, où l'amine secondaire est sélectionnée dans le groupe consistant en les suivantes : diéthylamine, dibutylamine, diéthalolamine, méthyléthylamine, di-n-propanolamine, iso-propanolamine, N-méthyléthanolamine, diéthylènetriamine, N-éthyléthanolamine, N-méthyléthanolamine, di-isopropanolamine et combinaisons de celles-ci, éventuellement où l'amine secondaire comprend la diéthalolamine, en outre éventuellement où l'amine secondaire comprend la diéthylènetriamine.

7. Procédé selon la revendication 4, où l'amine tertiaire est sélectionnée dans le groupe consistant en les suivantes : N,N-diméthyléthanolamine, triéthylamine, triméthylamine, triisopropylamine, méthyldiéthanolamine, triéthanolamine et combinaisons de deux ou plusieurs de celles-ci, éventuellement où l'amine tertiaire comprend la N,N-diméthyléthanolamine.

8. Procédé selon la revendication 4, où l'amine quaternaire comprend une amine quaternaire polymère répondant à la formule générale : où :
R¹, R², R³ et R⁴ peuvent indépendamment être identiques ou différents et peuvent être sélectionnés parmi -CH₃, -CH₂CH₃, -CH(CH₃)₂ ou -CH₂CH₂OH ;
R⁵ représente -CH₂CH₂-, -CH₂CH₂CH₂-, -CH₂CH₂CH₂CH₂-, -CH₂CHOHCH₂- ou -CH₂CH₂OCH₂CH₂ ;
X et Y peuvent être identiques ou différents et sont sélectionnés parmi Cl, Br et I ;
v et u peuvent être identiques ou différents et peuvent chacun prendre une valeur qui va de 1 à 7 ; et
n prend une valeur qui va de 2 à 200, éventuellement où, dans l'amine quaternaire polymère,
R¹, R², R³ et R⁴ représentent chacun -CH₃ ;
R⁵ représente -CH₂CH₂OCH₂CH₂ ;
v et u prennent la valeur 3 ;
X et Y représentent Cl ; et
n est une moyenne de 6.

9. Procédé selon la revendication 1 où la concentration en amine et/ou en ammoniaque dans la solution de conditionnement est entre 5 et 100g/l, éventuellement où la concentration en amine et/ou en ammoniaque dans la solution de conditionnement est entre 10 et 50 g/l.

10. Procédé selon la revendication 1, où le pH de la solution de conditionnement est entre 0 et 14, éventuellement où le pH de la solution de conditionnement est entre 6 et 12.

11. Procédé selon la revendication 1, comprenant en outre l'étape de mise en contact du substrat en plastique activé avec un traitement acide avant l'étape (d).
